

# UNITED STATES PATENT OFFICE.

HANS LÜTTKE, OF HAMBURG, GERMANY.

## PHOTOGRAPHIC EMULSION AND PROCESS OF MAKING SAME.

SPECIFICATION forming part of Letters Patent No. 722,238, dated March 10, 1903.

Application filed October 16, 1901. Serial No. 78,793. (No specimens.)

*To all whom it may concern:*

Be it known that I, HANS LÜTTKE, a citizen of Prussia, and a resident of Hamburg, Germany, have invented certain new and useful 5 Improvements in Photographic Emulsions and Processes of Making the Same, of which the following is a specification.

My invention relates to the manufacture of light-sensitive emulsions such as are used for 10 coating printing-out paper. Such papers as a rule are coated with an emulsion containing silver chlorid, and it is well known that the tint or color obtained by simply fixing the print is unsatisfactory and that for this 15 reason a separate operation called "toning" is generally resorted to for the purpose of giving the image an agreeable tone. The toning solutions generally contain gold salts. Attempts have been made to incorporate gold 20 salts with the emulsion, so that the prints might be fixed at once without a separate toning operation. These attempts, however, have so far failed to accomplish a thoroughly 25 satisfactory result.

I have made extensive experiments, and as 30 a result of this investigation I have come to the conviction that the reason of the failure experienced so far is the employment of chlorids, either of gold alone or gold in connection with alkalies. When such salts are used, the chlorin combines with the silver, and a gold compound is formed and precipitated which is not available for toning purposes. I have found that gold compounds containing 35 no chlorin are required to avoid the defects hitherto observed and that the following substances are particularly well suited for the intended purpose: auryl sulfate,  $(Au(OH)HSO_4)$ , auri nitrate nitric acid,  $Au(NO_3)_3$ ,  $+HNO_3+3H_2O$ , as well as the alkali double 40 salts of these compounds, and principally the double salt of lithium. When employing emulsions containing these gold salts, an image is produced which consists not only of 45 reduced silver, but also of reduced gold. The toning process therefore takes place simultaneously with the printing, and subsequent toning such as now practiced is dispensed with.

50 I find that the best results are obtained if the emulsion contains a proportion of silver chlorid equal to from thirty to fifty per cent. of the entire quantity of silver. I find that

the reduced silver which has been produced by exposing to light mixtures containing silver chlorid, silver nitrate, and silver citrate has in a very high degree the property of reducing gold.

As an example of my invention I will give the following receipt for an emulsion: (A) Celloidin collodion, four per cent., six hundred and twenty cubic centimeters; ether, 0.720, one hundred cubic centimeters; alcohol, ninety-six per cent., thirty cubic centimeters. (B) Silver nitrate, twenty-five grams; water, twenty-five cubic centimeters; alcohol, one hundred and twenty cubic centimeters; gold and lithium nitrate, 1.4 grams; auryl sulfate, 0.9 grams; lithium auryl sulfate, 1.3 grams. (C) Calcium chlorid, (anhydrous,) three grams, or lithium chlorid, (anhydrous,) three grams. (D) Citric acid, five grams; alcohol, thirty cubic centimeters.

It will be understood that the collodion is used as a binder and that instead of this I 75 may employ equivalent substances, as gelatin, albumen, and starch.

I may employ gold nitrates or sulfates, as hereinbefore described, as equivalents, and while in the claims I refer to the sulfates 80 only I desire it to be understood that the employment of a gold nitrate is to be considered covered as an equivalent.

Having described my invention, what I 85 claim, and desire to secure by Letters Patent, is—

1. The process of producing photographic emulsions, which consists in adding a gold sulfate to an argentic emulsion.

2. The process of producing photographic 90 emulsions, which consists in adding a gold sulfate to an argentic emulsion and chemically binding to chlorin from thirty to fifty per cent. of the total amount of silver contained in the emulsion.

3. An argentic photographic emulsion, said 95 emulsion containing a gold sulfate.

4. An argentic photographic emulsion, said 100 emulsion containing a gold sulfate and having from thirty to fifty per cent. of the entire silver contents chemically combined with chlorin.

HANS LÜTTKE.

Witnesses:

E. H. L. MUMMENHOFF,  
OTTO W. HELLMRICH.